

1

2,891,010

**WATERPROOF SILICA-BASE GREASES**

Thomas W. Martinek, Crystal Lake, Ill., assignor to The Pure Oil Company, Chicago, Ill., a corporation of Ohio

No Drawing. Application December 7, 1955  
Serial No. 551,509

4 Claims. (Cl. 252—28)

This invention relates to the thickening of oleaginous liquids by means of finely divided, inorganic gelatinous material. It is especially directed to the preparation of water-resistant lubricants comprising an oleaginous vehicle thickened to a grease-like consistency with a non-soap inorganic gelling agent for use in high temperature applications.

Although lubricating greases by ASTM definition are semi-solid or solid combinations of a petroleum product and a soap or a mixture of soaps, there have been developed a number of compositions which do not employ petroleum oils as the base constituent and a number of thickeners for these base liquids which are non-soap gelling agents, but can be used in the preparation of thickened compositions which functionally are the equivalents of a true lubricating grease. Furthermore, the lubricating compositions thus prepared have properties in which soap-containing petroleum base lubricating greases are generally deficient. In spite of the fact that the compositions of this invention do not conform with the conventional definition of a grease, they will hereinafter be included in this category in order to facilitate the discussion of the instant invention.

Inorganic colloids capable of gel formation in oleaginous vehicles include alkaline earth metal oxides and hydroxides; carbonates of alkali metal and alkaline earth metals, ferric oxide, vanadium pentoxide, oxides and hydroxides of polyvalent metals, such as silicon, magnesium, aluminum, tin, chromium, etc.; sulfides of polyvalent metals including cuprous sulfide, ferrous sulfide, and others. The preparation of inorganic colloidal thickening agents is comprehensively discussed in the patent literature. For examples, see U.S. Patents 2,260,645, 2,583,603—4, 2,554,222, 2,594,822, 2,629,691, and others. Also included are the siliceous gelling agents prepared by pyrolyzing silicon compounds, such as silicon tetrachloride, tetraethyl silicate, or a chlorosilane to produce finely divided materials. Examples of this type of gelling agent are the Cab-O-Sils marketed by the Godfrey L. Cabot, Inc.

A non-soap gelling agent which has found considerable application in the preparation of lubricating greases is finely-divided silica. Accordingly, the following discussion is directed to a description of greases prepared by the use of this material. However, this is only illustrative and non-limiting. This material, when dispersed in a suitable liquid medium including petroleum oil lubricating fractions, will produce a gelatinous composition with a grease-like structure having lubricating properties. The development of inorganic gelling agents apparently originated in Germany during World War II as a solution to

2

the shortage of conventional grease-making components. Greases employing inorganic gelling agents can be prepared in the standard type of grease-making equipment without requiring unusual processing conditions. Although the greases thickened with inorganic gelling agents are suitable for multi-service duty, their resistance to changes in consistency over a wide temperature range makes them very desirable compositions for high temperature applications. While the consistency of soap-thickened greases at elevated temperature is inimicably affected, greases thickened with inorganic gelling agents retain their grease structure. If working of these greases has occurred, the base oil may distill or even ignite, but no melting of the grease results. Unfortunately, these multi-purpose greases do not present an ideal solution to lubricating problems inasmuch as one serious deficiency in greases thickened with inorganic gelling agents is demonstrated by their lack of water resistance. This characteristic is fatal because exposure of a simple admixture of silica and oil to water results in the rapid disintegration of the mixture into its component parts. It has been found, however, that by treating the gelling agents employed in the preparation of lubricating greases with suitable reagents, the inorganic gel-oil composition can be stabilized against the detrimental effect of water. Improvement in the water resistance is effected by coating the inorganic gelling agent or by using suitable additives in the lubricating grease. Boner, in Manufacturing and Application of Lubricating Greases, Reinhold, 1954, at page 704, et seq., comprehensively discusses the modification of silica gel to increase water resistance based on a compilation of the prior art.

Various methods are employed to evaluate the resistance to breakdown of the grease structure in the presence of water. One technique involves the addition of incremental amounts of water with subsequent mixing of the water-lubricant system, and observation of the accompanying change in grease structure, if any. Another test immerses a sample of the grease, retained in a suitable specimen holder, into boiling water for one-half hour. Apparently a more rigorous procedure for determining the water resistance of a grease of this nature is the test method ASTM designation: D1264-53T, described in the 1953 Supplement to Book of ASTM Standards, Part 5, ASTM. In this method the grease sample is retained in a rotating ball bearing and subjected to the washing action of distilled water for 1 hour at specified test temperatures. It has been found that waterproofing agents generally considered adequate for imparting water resistance to water-susceptible greases prepared from inorganic gelling agents are unsatisfactory for making a grease composition which will give satisfactory results, when subjected to the scrutiny of the aforementioned ASTM method for determining the water washout characteristics of a lubricating grease.

It is therefore an object of this invention to provide a non-soap-thickened lubricating grease having enhanced water resistance. Another object of this invention is the production of a lubricating grease having improved resistance to water washout. It is also an object of this invention to improve the water washout characteristics of a silica-thickened lubricating grease. These and other objects will become apparent from the following detailed description of this invention.

According to this invention, it has been found that in

order to provide a non-soap-thickened lubricating grease having excellent resistance to water washout, it is necessary to incorporate in the grease composition a combination waterproofing additive comprising an admixture of (1) an oil-soluble alkylaryl polyether alcohol prepared by condensing an alkyl phenol and ethylene oxide, and (2) an oil-soluble aliphatic monoether or polyoxyalkylene glycol prepared by the addition of a monohydroxy aliphatic alcohol to 1,2-propylene oxide.

In formulating the grease composition of this invention

ration of suitable compositions are reported in U.S. Patent 2,448,664. Although a variety of monohydric aliphatic alcohols can be employed in the reaction, preferred compositions are prepared by reacting butanol and 5 1,2-propylene oxide. By varying the molecular weight of the addition product, changes in product characteristics are obtained, as shown in Table I, wherein are tabularly summarized the properties of proprietary compositions of this nature marketed by Carbide and Chemicals Corporation under the mark "Ucon."

TABLE I  
Properties of Ucon brand lubricants—LB series

|                                         | LB-140  | LB-300    | LB-400    | LB-550    | LB-650  |
|-----------------------------------------|---------|-----------|-----------|-----------|---------|
| Viscosity, SUS at:                      |         |           |           |           |         |
| 210 F.                                  | 45.5    | 62.7      | 74.3      | 91.9      | 107     |
| 100 F.                                  | 140     | 300       | 400       | 550       | 650     |
| 0 F.                                    | 4,960   | 18,380    | 27,600    | 40,800    | 50,500  |
| -30 F.                                  | 42,100  | 183,000   | 284,000   | 444,000   | 540,000 |
| -50 F.                                  | 265,000 | 1,370,000 | 2,335,000 | 3,890,000 | -----   |
| Viscosity, centistokes at:              |         |           |           |           |         |
| 210 F.                                  | 5.9     | 11.0      | 14.1      | 18.5      | 22.0    |
| 100 F.                                  | 29.8    | 65.0      | 86.6      | 119       | 141     |
| 0 F.                                    | 1,080   | 4,000     | 6,000     | 8,000     | 11,000  |
| -30 F.                                  | 9,200   | 40,000    | 62,000    | 97,000    | 118,000 |
| -50 F.                                  | 58,000  | 300,000   | 510,000   | 850,000   | -----   |
| V.I. (ASTM D-587-41)                    | 147     | 142       | 142       | 140       | 140     |
| Pour Point (ASTM D-97-39), F.           | -50     | -40       | -35       | -30       | -25     |
| Density at 210 F., g. per cc.           | 0.921   | 0.933     | 0.936     | 0.939     | 0.940   |
| Density at 100 F., g. per cc.           | 0.966   | 0.979     | 0.983     | 0.985     | 0.986   |
| Specific Gravity at 60 F.               | 0.983   | 0.997     | 1.001     | 1.003     | 1.004   |
| Gravity, deg. API at 60 F.              | 12.5    | 10.5      | 9.7       | 9.5       | 9.4     |
| Flash Point (ASTM D-92-33), F.          | 440     | 470       | 485       | 510       | 525     |
| Fire Point (ASTM D-92-33), F.           | 510     | 570       | 580       | 580       | 580     |
| Carbon Residue (ASTM D-189-45), percent | (1)     | (1)       | (1)       | (1)       | (1)     |
| Ash (ASTM D-482-43-T), percent          | (1)     | (1)       | (1)       | (1)       | (1)     |

<sup>1</sup> Less than 0.01.

tion, a suitable inorganic gelling agent such as those described above, preferably silica aerogel, which has been prepared according to the method of Kistler in U.S. Patent 2,260,625, is incorporated in a selected oleaginous vehicle including conventional mineral lubricating oils of Pennsylvania, Mid-Continent, Gulf Coast, East Texas, California, etc. origin. Other oleaginous bases may also be employed, such as synthetic lubricating oil derived from the polymerization of olefinic charge stocks; aliphatic and aromatic esters, viz., aliphatic esters of dicarboxylic acids, e.g., diethyl sebacate; organic phosphates, e.g., tricresyl phosphate; silicone oils, and other oleaginous liquid possessing satisfactory lubricity characteristics. To impart to the finished grease satisfactory water washout resistance, the waterproofing additive of this invention is admixed with the oil-thickener blend. This oil-soluble additive consists of a combination of (1) an alkyl aryl polyether alcohol, and (2) an aliphatic monoether of a polyoxyalkylene glycol.

The polyether alcohol constituent of the waterproofing additive is prepared by condensing an alkyl phenol with ethylene oxide to form an oil-soluble product having a molecular weight of about 200-550. Phenols having C<sub>1</sub>-C<sub>18</sub> alkyl substituents, such as di-isobutyl phenol, octyl phenol, nonyl phenol, octadecyl phenol, tridecyl phenol, diethyl phenol, and others, or mixtures thereof, can be condensed according to conventional techniques with ethylene oxide to provide polyether alcohols of molecular weight sufficient to impart oil solubility characteristics to the polyether alcohol. An example of a preferred alkyl aryl polyether alcohol is Triton X-45, a proprietary compound marketed by Rohm and Haas Company.

The other constituent of the waterproofing additive is an oil-soluble aliphatic monoether of a polyoxyalkylene glycol which is synthesized by adding a monohydroxy aliphatic alcohol to propylene oxide. Details for prepa-

40 For the compositions of this invention, it is preferred that the aliphatic monohydric alcohol-propylene oxide addition product having an average molecular weight of about 800-1600 (acetyl value) be employed. According to this invention, the combination of (1) an oil-soluble additive product of an aliphatic monohydric alcohol and propylene oxide, and (2) an oil-soluble alkyl aryl polyether alcohol, in the ratio of 1 to 15 parts by weight of the former to one part by weight of the latter, will improve the water washout characteristics of a non-soap-thickened grease. It is preferred that a ratio of 4-8:1 be employed to give optimum results. The amount of 45 composite additive employed will depend upon the amount of gelling agent used. Generally, 9 to 10% by weight, based on gelling agent, will provide satisfactory results. However, amounts outside this range may be employed. In order to prepare a finished grease it may be necessary 50 to add other functional additives to impart to the finished grease corrosion and oxidation resistance, extreme pressure characteristics, etc. Table II shows illustrative ranges of ingredients.

TABLE II

| Component                                                                          | Parts by Weight |             |
|------------------------------------------------------------------------------------|-----------------|-------------|
|                                                                                    | Suggested       | Preferred   |
| Liquid, oleaginous lubricating vehicle                                             | 80-96           | 88-94       |
| Non-soap gelling agent                                                             | 4-20            | 6-12        |
| Water-proofing additive                                                            | 3-2.0           | .5-1.1      |
| Functional additive, e.g., rust inhibitor, anti-oxidant, V.I. improver, E.P. agent | As required     | As required |

70 The subject invention is illustrated in a non-limited manner by the tabular summary of data shown in Table III.

TABLE III

| Composition, Wt., Percent                                                                             | A     | B     | C     | D     | E     | F     | G     | H     | I     | J     | K     | L    | M     | N     |
|-------------------------------------------------------------------------------------------------------|-------|-------|-------|-------|-------|-------|-------|-------|-------|-------|-------|------|-------|-------|
| Silica Aerogel Thickener <sup>1</sup>                                                                 | 9.0   | 9.0   | 9.0   | 9.0   | 9.0   | 9.0   | 9.0   | 9.0   | 9.0   | 9.0   | 9.0   | 9.0  | 9.0   | 9.0   |
| Waterproofing Agent:                                                                                  |       |       |       |       |       |       |       |       |       |       |       |      |       |       |
| Aliphatic monoether of polyoxyalkylene glycol <sup>2</sup>                                            | 0.72  | 0.74  | 0.65  | 0.80  | 0.56  | 0.92  | 0.36  |       | 0.45  | 0.63  |       |      | 0.64  | 0.80  |
| Alkyl aryl polyether alcohol <sup>3</sup>                                                             | 0.09  | 0.074 | 0.16  | 0.05  | 0.18  |       | 0.27  | 0.45  |       |       | 0.63  | 0.9  | 0.08  | 0.10  |
| Ratio:                                                                                                |       |       |       |       |       |       |       |       |       |       |       |      |       |       |
| Aliphatic monoether of polyoxyalkylene glycol <sup>2</sup> /alkyl aryl polyether alcohol <sup>3</sup> | 8     | 10    | 4     | 16    | 3.1   |       | 1.3   |       |       |       |       |      | 8     | 8     |
| Waterproofing Agent <sup>4</sup>                                                                      |       |       |       |       |       |       |       |       |       |       |       |      |       |       |
| 100 Silica Aerogel                                                                                    | 9     | 9     | 9     | 9.4   | 8.2   | 10    | 5     | 5     | 7     | 7     | 10    | 8    | 10    |       |
| Mineral Lubricating Oil <sup>5</sup>                                                                  | 90.19 | 90.19 | 90.19 | 90.15 | 90.26 | 90.08 | 90.37 | 90.55 | 90.55 | 90.37 | 90.37 | 90.1 | 90.28 | 90.10 |
| Grease Characteristics:                                                                               |       |       |       |       |       |       |       |       |       |       |       |      |       |       |
| Penetration <sup>6</sup>                                                                              |       |       |       |       |       |       |       |       |       |       |       |      |       |       |
| Unworked                                                                                              | 249   | 235   | 237   | 233   | 239   | 241   | 250   | 255   | 238   | 249   | 248   | 249  | 239   | 238   |
| Worked                                                                                                | 282   | 262   | 259   | 271   | 257   | 275   | 275   | 309   | 275   | 264   | 313   | 282  | 276   | 265   |
| Water Washout <sup>6</sup> wt. percent grease loss                                                    | 15    | 21    | 15    | 39    | 26    | 39    | 22    | 41    | 56    | 59    | 25.2  | 84.1 | 60.4  | 24.3  |

<sup>1</sup> Santocel ARD, a proprietary silica aerogel marketed by Monsanto Chemical Company, having a particle size of 3-5 microns in diameter, a bulk density of 0.056-0.064 gms./ml.

<sup>2</sup> UCON-LB 550, a proprietary composition marketed by Carbide and Carbon Chemicals comprising an oil-soluble addition product of butanol and 1,2-propylene oxide having an average molecular weight of about 1,400 (acetyl value) and having the characteristics shown in Table I.

<sup>3</sup> Triton X-45, a proprietary compound marketed by Rohm and Haas Company, comprising an oil-soluble admixture of homologous polyether alcohols having an average molecular weight of 338-514 and prepared by condensing di-isobutyl phenol and ethylene oxide.

<sup>4</sup> Intermediate V.I. bright stock mineral lubricating oil prepared by phenol extracting, MEK dewaxing, and clay contacting a Mid-Continent lubricating oil fraction, and having the following characteristics:

|                           |  |  |  |  |  |  |  |  |  |  |  |  |  |       |
|---------------------------|--|--|--|--|--|--|--|--|--|--|--|--|--|-------|
| Viscosity, SUS at 210°    |  |  |  |  |  |  |  |  |  |  |  |  |  | 16.4  |
| Gravity, API <sup>7</sup> |  |  |  |  |  |  |  |  |  |  |  |  |  | 24.5  |
| Flash, °F. (COC)          |  |  |  |  |  |  |  |  |  |  |  |  |  | 565   |
| Fire, °F. (COC)           |  |  |  |  |  |  |  |  |  |  |  |  |  | 630   |
| Viscosity Index           |  |  |  |  |  |  |  |  |  |  |  |  |  |       |
| Pour point, °F. ASTM      |  |  |  |  |  |  |  |  |  |  |  |  |  | 91    |
| Color NPA (ASTM)          |  |  |  |  |  |  |  |  |  |  |  |  |  | 0     |
| Carbon residue, percent   |  |  |  |  |  |  |  |  |  |  |  |  |  | 7     |
| Sulfur, percent           |  |  |  |  |  |  |  |  |  |  |  |  |  | 1.20  |
| Neut. No. (I)             |  |  |  |  |  |  |  |  |  |  |  |  |  | 0.80  |
| Ash, percent              |  |  |  |  |  |  |  |  |  |  |  |  |  | 0.05  |
|                           |  |  |  |  |  |  |  |  |  |  |  |  |  | 0.002 |

<sup>5</sup> ASTM Designation D 128-47.

<sup>6</sup> ASTM Designation D 1264-53T.

The effectiveness of the instant invention for enhancing the water washout characteristics of a non-soap-thickened lubricating grease is further illustrated by comparison with a lithium soap-thickened lubricating grease having the following composition:

| Component                                                                                                     | Wt. Percent |
|---------------------------------------------------------------------------------------------------------------|-------------|
| Lithium 12-hydroxy stearate                                                                                   | 8           |
| Mineral oil base:                                                                                             |             |
| Intermediate V.I. (160 S.U.S. at 210° F./90 V.I.) Mid-Continent solvent-refined, bright stock lubricating oil | 87          |
| High V.I. (85 S.U.S. at 100° F./95 V.I.) Mid-Continent, solvent-refined, neutral lubricating oil              | 8           |
| Phenol extract of a bright stock lubricating oil fraction <sup>1</sup>                                        | 5           |

<sup>1</sup> A mineral oil lubricating fraction obtained as an extract from the phenol extraction of a dewaxed and deasphalted Mid-Continent residue and having the following characteristics:

|                                        |               |
|----------------------------------------|---------------|
| API gravity                            | 14.0          |
| Viscosity:                             |               |
| S.U.S. at 100° F                       | 27,000 (ext.) |
| S.U.S. at 210° F                       | 369           |
| Viscosity Index                        | 26            |
| Pour point, °F                         | +65           |
| Conradson carbon residue (wt. percent) | 4.54          |

## PROPERTIES

|                                                         |      |
|---------------------------------------------------------|------|
| Worked penetration <sup>2</sup>                         | 268  |
| Water washout <sup>3</sup> , weight percent grease loss | 18.3 |

<sup>2</sup> ASTM designation D128-47.

<sup>3</sup> ASTM designation D1264-53T.

It will be seen that, by means of this invention, a non-soap-thickened lubricating grease can be made, which will have water washout characteristics comparable to a lithium soap-thickened lubricating grease, a composition to which is generally attributed good water resistance, and is used as a multi-purpose lubricant. To further illustrate the advantages of the instant invention, a non-soap-thickened lubricating grease was prepared without employing the composite water-proofing agent of this invention. It was found that this grease had no resistance to water washout and completely disintegrated under the water washout test conditions.

I claim as my invention:

1. A silica-thickened grease having enhanced water washout characteristics consisting essentially of a lubricating oil having incorporated therein a finely divided silica gelling agent in an amount sufficient to impart a grease-like consistency to said lubricating oil, and a composite water-proofing agent consisting essentially of 4-10 parts by weight of (1) an oil-soluble mono-alkyl ether of a polyoxyalkylene glycol produced by reaction of a monohydric aliphatic alcohol and 1,2-propylene oxide having a molecular weight of 800-1600 (acetyl value), and one part by weight of (2) an oil-soluble mono-alkylaryl ether of a polyoxyethylene glycol produced by reaction of a C<sub>1</sub>-C<sub>18</sub> alkyl-substituted phenol and ethylene oxide having an average molecular weight of 200-550, said waterproofing agent being present to the extent of 9-10% by weight of the silica in an amount sufficient to improve substantially the water-washout characteristics of said grease.

2. A grease composition in accordance with claim 1 in which the composite waterproofing agent contains 4-8 parts by weight of compound (1) and one part by weight of compound (2), said waterproofing agent representing about 9% by weight of the silica.

3. A silica-thickened lubricating grease composition consisting essentially of:

| Components                                                                                                                                                                                                            | Parts by Weight |
|-----------------------------------------------------------------------------------------------------------------------------------------------------------------------------------------------------------------------|-----------------|
| Mineral lubricating oil                                                                                                                                                                                               | 90              |
| Finely divided silica                                                                                                                                                                                                 | 9               |
| Waterproofing Additive:                                                                                                                                                                                               |                 |
| a. An oil-soluble mono-alkyl ether of a polyoxyalkylene glycol produced by reaction of a monohydric aliphatic alcohol and 1,2-propylene oxide having a molecular weight of 800-1,600 (acetyl value)                   | 0.65-0.75       |
| b. An oil-soluble mono-alkyl aryl ether of polyoxyethylene glycol produced by reaction of a C <sub>1</sub> -C <sub>18</sub> alkyl-substituted phenol and ethylene oxide having an average molecular weight of 200-550 | 0.07-0.16       |

4. A silica-thickened lubricating grease composition consisting essentially of:

| Components                                                                                                                                                                                                             | Parts by weight |
|------------------------------------------------------------------------------------------------------------------------------------------------------------------------------------------------------------------------|-----------------|
| Mineral lubricating oil                                                                                                                                                                                                | 5               |
| Finely-divided silica                                                                                                                                                                                                  | 90              |
| Waterproofing Additive:                                                                                                                                                                                                |                 |
| a. An oil-soluble mono-alkyl ether of a polyoxyalkylene glycol produced by reaction of a monohydric aliphatic alcohol and 1,2-propylene oxide having a molecular weight of 800-1,600 (acetyl value).                   | 0.80            |
| b. An oil-soluble mono-alkyl aryl ester of polyoxyethylene glycol produced by reaction of a C <sub>1</sub> -C <sub>18</sub> alkyl-substituted phenol and ethylene oxide having an average molecular weight of 200-550. | 0.10            |

## References Cited in the file of this patent

## UNITED STATES PATENTS

|                 |                |
|-----------------|----------------|
| Peterson        | Oct. 30, 1951  |
| Moore et al.    | Sept. 15, 1953 |
| Hotten et al.   | June 1, 1954   |
| Weihe et al.    | May 20, 1956   |
| Marshall et al. | Oct. 9, 1956   |